

## UNITED STATES PATENT OFFICE

FRITZ HOFMANN, OF BRESLAU, AND MANFRED DUNKEL, OF MANNHEIM, GERMANY,  
ASSIGNORS TO I. G. FARBENINDUSTRIE AKTIENGESELLSCHAFT, OF FRANKFORT-  
ON-THE-MAIN, GERMANY, A CORPORATION OF GERMANY

## PRESERVATION OF OILS

No Drawing. Application filed June 14, 1928, Serial No. 285,499, and in Germany November 24, 1925.

The present invention relates to the preservation of oils against oxidation.

We have found that oils, especially lubricating and transformer oils, and in particular hydrocarbon oils can be preserved from the obnoxious action of atmospheric oxygen at elevated temperatures and the discoloration of the oils and the formation of asphalt-like sludge prevented by the addition of small amounts of non-gaseous nitriles which are soluble in the said oils.

The said nitriles may also be employed in admixture with other organic substances such as bases, aldehydes and their condensation products, acid amides and their derivatives and the like.

The following examples serve to illustrate our invention which, however, is not limited thereto. The percentages are by weight.

*Example 1*

On addition to a mineral oil, which on oxidation yields 0.45 per cent of tarry matter, of 0.1 per cent of acetonitrile only 0.04 per cent of tarry matter are obtained by a similar treatment.

*Example 2*

30 The same oil when mixed with 0.1 per cent of toluo-nitrile yields only 0.03 per cent of tarry matter.

This application is a continuation in part of the application for Letters Patent, Ser. 35 No. 145,098, filed Oct. 29, 1926.

What we claim is:

1. A composition of matter comprising a lubricating oil and 0.1 per cent by weight of toluo-nitrile.

40 2. The process of preserving oils from the obnoxious action of oxygen which comprises adding to the oils a small amount of toluo-nitrile.

3. The process of preserving a hydrocarbon oil from the obnoxious action of oxygen which comprises adding to said oil a small amount of toluo-nitrile.

45 4. The process of preserving an oil of the type used for lubricating and in transformers from the obnoxious action of oxygen

which comprises adding to said oil about 0.1 per cent by weight of toluo-nitrile.

5. A composition of matter comprising an oil and a small amount of toluo-nitrile.

6. A composition of matter comprising a hydrocarbon oil and a small amount of toluo-nitrile.

In testimony whereof we have hereunto set our hands.

FRITZ HOFMANN.  
MANFRED DUNKEL.

30

65

70

75

80

85

90

100